

Patented Mar. 10, 1925.

1,529,083

# UNITED STATES PATENT OFFICE.

SAMUEL PEACOCK, OF WHEELING, WEST VIRGINIA, ASSIGNOR TO WHEELING STEEL & IRON COMPANY, OF WHEELING, WEST VIRGINIA, A CORPORATION OF WEST VIRGINIA.

## PROCESS OF COATING IRON AND STEEL SHAPES WITH OTHER METALS.

No Drawing.

Application filed June 7, 1922. Serial No. 566,657.

To all whom it may concern:

Be it known that I, SAMUEL PEACOCK, a citizen of the United States, residing at Wheeling, in the county of Ohio and State 5 of West Virginia, have invented certain new and useful Improvements in Processes of Coating Iron and Steel Shapes with Other Metals; and I do hereby declare the following to be a full, clear, and exact description 10 of the invention, such as will enable others skilled in the art to which it appertains to make and use the same.

This invention relates to a process of coating iron or steel shapes in general with 15 other metals and alloys and has for its object to improve as well as to lessen the cost of the processes heretofore proposed.

With these and other objects in view the invention consists in the novel steps and 20 combinations of steps constituting the process, all as will be more fully hereinafter disclosed and particularly pointed out in the claims.

It is well known that steel and iron 25 shapes, such, for example, as plates and other iron and steel objects, have been heretofore coated with tin, copper, and other metals by various electrolytic processes, but it is also well known that if the coating 30 metal or alloy is too rapidly deposited it will be more or less pulverulent, porous or fluffy in character, and therefore non-adherent and worthless for protective purposes. On the other hand, it is equally well 35 known that the relatively slow and tedious process of making a coherent, firm, tenacious, and satisfactory coating by processes now available is relatively so costly that iron and steel coated articles are not as freely 40 used as they would be if this cost could be reduced.

The required time and fine adjustments of the various factors of the prior processes contribute largely to the items of cost of 45 coating one metal with another, which it is the object of this invention to reduce.

In carrying out this invention for the deposition of tin on steel, for example, I may 50 provide coating solutions of stannous chloride and ammonium alum of the usual concentrations employed in electroplating processes, or in chemically depositing processes, or I may somewhat increase their concentrations. I prefer however to employ a

suitable so called restraining agent, or addition agent, as I find it improves the final product.

Having provided a tin coating solution, I next deposit the tin on the steel or iron object to be coated, as by electrodeposition 60 or by straight chemical deposition but in carrying out this process, I do not have to remove the black ferro-ferric oxide which usually coats such articles, and especially coats sheets of steel, immediately after they 65 leave the furnace. As is well known, the cost of removing this ever-present black oxide coating in the making of so called "tin plate" constitutes a large item of the total cost of the process. Further, instead 70 of causing the deposition of the tin coating to be gradually effected as was necessary in the prior procedures to obtain a firm and coherent deposit, I cause the coating to be deposited relatively very rapidly, so that 75 it appears in a more or less pulverulent, porous, and non-adhering form. This form in the prior procedures would not be suitable at all for the purpose in hand, but in this process it is highly suitable in that it 80 serves to get the requisite amount of tin in contact with the steel in a minimum of time, and without having to adjust such factors as purity of solution; temperature of deposition, concentration, etc., all of 85 which are annoying and cost money in large scale operations. But, of course, I maintain the strength of the solution fairly constant by the usual stirring means and by the presence of undissolved tin, or tin 90 salts in the solution.

Having thus secured a porous coating of tin on the oxidized surface of a sheet of steel, for example, in a relatively very short time, I next wash and dry the coated sheet 95 in the usual manner, when it will be found to possess a dull surfaced coating which is non-crystalline, porous, and easily rubbed or scratched off. I have found that the particles of this porous coating may be fritted 100 together and made to adhere to the surface of the steel sheet or plate at a temperature which is say 200° F. below the melting point of the tin itself. Accordingly, I next suitably heat up the coated steel plate to 105 about 250° F. The oxygen which was present in the ferro-ferric oxide coating of the steel sheet will be found to have been used

up in oxidizing a portion of the tin in the solution, so that the remaining tin will now enter the non-oxidized, or reduced surface of the steel sheet, or plate, and form a firm, 5 tenacious and exceedingly coherent protecting film of tin of the highest quality. The finished product, if it is to be used for tin cans is next polished or further treated as in the prior processes.

- 10 5 In case copper is to be deposited on steel sheets, or other iron or steel shapes, substantially the same procedure is carried out except a solution of copper sulphate is preferably employed, and the porous coating is 15 fritted together at a temperature of, say, 300° C. below the melting point of the copper. In the case of nickel, this temperature is about 400° C. below the melting point of the nickel.
- 20 25 Alloys are deposited in the same general way as that outlined for tin. That is, a porous relatively non-adherent coating of the alloy on the steel sheet is produced in the manner well known, when it is fritted together at a temperature well below its melting point, but sufficiently high to cause the constituents of the coating present to remove any remaining oxide on the steel surface to be coated, to the end that the coating 30 35 material will deposit on a clean surface before said surface has a chance to be re-oxidized.

The heating process should be carried out in a non-oxidizing atmosphere. Wherever 35 40 the term "metal" or "metals" occur in the claims, and refer to the coating material it is to be understood that metal alloys are to be included.

It is obvious that those skilled in the art 40 45 may vary the details of the process, without departing from the spirit of the invention, and therefore I do not wish to be limited to the foregoing disclosure except as may be required by the claims.

45 50 What is claimed is:

1. The process of coating iron and steel shapes with other metals which consists in

covering the surfaces to be protected when in an oxidized condition with a porous and relatively non-adherent deposit of the coating metal from a solution; and by the aid of heat converting said deposit into a partially oxidized non-porous and adherent protecting film on said surfaces, substantially as described. 55

2. The process of coating iron and steel shapes with other metals which consists in covering the surfaces to be protected when in an oxidized condition with a porous and relatively non-adherent deposit of the coating metal from a solution containing an addition agent; and by the aid of heat converting said deposit into a partially oxidized non-porous and adherent protecting film on said surfaces, substantially as described. 60

3. The process of coating the surfaces of iron and steel shapes with another metal which consists in covering said surfaces when in an oxidized condition with a solution of the coating metal; depositing out said metal onto said surfaces in a relatively porous and non-adherent film; and raising the temperature to a point sufficient to frit together the particles of said coating and to 70 75 provide a relatively non-porous adherent protecting film on the objects coated, substantially as described.

4. The process of coating the surfaces of iron and steel shapes with another metal 80 which consists in covering said surfaces when in an oxidized condition with a solution of the coating metal; depositing out said metal onto said surfaces in a relatively porous and non-adherent film; and raising 85 the temperature in a non-oxidizing atmosphere to a point sufficient to partially frit together the particles of said coating and to provide a relatively non-porous adherent 90 protecting film on the objects coated, substantially as described.

In testimony whereof I affix my signature.

SAMUEL PEACOCK.